

Sept. 12, 1972

K. G. HORNING

3,690,811

ACID DYEING FOR TERTIARY AMINATED POLYAMIDE, POLYOLEFIN  
AND POLYAMIDE BLENDS AND DISPERSE DYEING OF  
SAID POLYOLEFIN AND POLYESTER BLENDS  
Filed June 1, 1970



Fig. 1



Fig. 2

Kermit G. Horning

INVENTOR.

BY *Emil W. Milan*

ATTORNEY

1

3,690,811

**ACID DYEING FOR TERTIARY AMINATED POLY-  
AMIDE, POLYOLEFIN AND POLYAMIDE  
BLENDs AND DISPERSE DYEING OF SAID  
POLYOLEFIN AND POLYESTER BLENDs**

Kermit G. Horning, Waynesboro, Va., assignor to Thiokol  
Chemical Corporation, Bristol, Pa.

Filed June 1, 1970, Ser. No. 42,357

Int. Cl. D06p 3/82

U.S. Cl. 8—21 B

14 Claims

**ABSTRACT OF THE DISCLOSURE**

A union dyed, solid colored, tufted carpeting, uniformly shaded in both the face yarns and in the backing material, comprises as the backing material woven ribbons of a composition comprising a polyolefin blended with a basic polyamide dye site additive, said additive consisting of a minor incorporated amount of a polyamide resin based on a linear aliphatic dicarboxylic acid and a polyamine containing two primary or secondary amine groups and at least one tertiary amine group.

**BACKGROUND OF THE INVENTION**

**Field of the invention**

This invention relates to a dyed tufted carpet in which both the carpet backing and the tufted face yarns are synthetic materials and are dyed to the same shade of the same color. Particularly, the invention relates to a synthetic fabric comprising a piece dyeable polypropylene-polyamide composition backing which dyes to a similar shade, described in the dyeing art as a union shade, in competition with tufted face yarns of nylon or polyester material, and wherein both the backing and the face yarns are dyed with the same acid or disperse dye in a single dye bath in a single dyeing operation.

**Description of the prior art**

The use of polypropylene filaments in ribbon or tape form interwoven to make a fabric which can be used as a backing material into which face yarns can be tufted to make a tufted carpet has become a widely practiced art. Tufted pile fabric comprising such a flat woven synthetic plastic backing is taught, for example, by T. M. Rhodes, U.S. Pat. 3,110,905. The synthetic materials used in making the backing and the face yarns are normally colorless or light beige colored materials which in themselves are unattractive for most fabric uses. Accordingly, dyeing of the materials ordinarily must be done to manufacture an attractive fabric. For example, the backing can be prepared from a ribbon filament which has been dyed by incorporation of a dye in the melted plastic material from which the filament is extruded. Also, the backing may be dyed after it has been woven into a fabric. The face yarn similarly may be dyed in its prefilamented or fibered form or after it has been formed into the yarn filament or fibered and twisted into a face yarn.

When a carpet manufacturer wishes to manufacture a solid colored tufted carpet using the synthetic carpet backing material, and a synthetic face yarn, he thus has several choices as to the colors of his starting materials. If he uses a previously dyed backing of a particular color and shade, he must then obtain a colored face yarn which

2

will match the color and shade of the backing. This selection is particularly critical if he is concerned about the backing showing through the face yarn. This concern in fact becomes a problem when tufted carpeting is applied over curved surfaces having sharp bends, such as the nosings on stairs. In such uses, the tufted carpeting is bent sharply, and even when it is densely tufted, the backing may show through the tufts of the yarn. Because the carpet tufters usually will be obtaining his backing material from one supplier and his face yarns from a different supplier, he may encounter considerable difficulty in obtaining a close match as to shade between the color of the face yarn and the color of the backing, particularly when he is tufting a carpet of a bright solid color, for example, a bright orange. Some carpet manufacturers are integrated in their operations to dye the carpet after it has been manufactured, and prefer to use an undyed face yarn in order to avoid stocking a large variety of colors of yarn, or for some other reason of economy. In the latter situation, the carpet manufacturer must be able to dye the face yarn to any desired color and shade. However, he also, in such case, may desire that the face yarn assume the same color and shade as the backing, so that the tufting need not be as dense as would be required to hide or minimize show-through when the carpeting is bent as discussed above. If both the carpet backing and the face yarn are used in an undyed condition in making the carpet and then are dyed simultaneously, it has been found that the face yarn and the backing material often do not dye to the same shade. This result may be due in part to the difference in sizes of the filaments or fibers of the face yarn as compared to the filaments of the backing, and the consequent optical effects which result, as well as in the difference in dye receptivities of a heavy thick ribbon and a thin fiber. For example, the backing for the tufted carpet is woven from large ribbon monofilaments of 500 to 1000 denier, whereas the face yarn may be formed of fine fibers of about 15 denier each.

Face yarns are usually derived from synthetic polymers, for example, polyamides, such as nylon, or polyesters, which have high dye affinity and which, accordingly, can be dyed readily to a wide variety of shades of color as well as to a wide variety of colors. On the other hand polypropylene, which is used mostly as a backing material and not as a face yarn, does not readily accept an organic dye. In order to overcome this disadvantage of polypropylene as a dyeable fabric material, a large variety of modified polypropylenes have been developed which makes the polypropylene composition thus formed a dyeable material. However, a modified polypropylene, while it accepts a dye, may not at the same time accept the dye in such a way and amount that it will assume the same shade of color as that of the face yarn which is tufted into the backing fabric, when the two are dyed simultaneously, in the same dye bath. The present invention overcomes this problem.

**SUMMARY OF THE INVENTION**

The present invention is directed to a dyed synthetic material fabric, particularly carpeting, in which the backing material comprises a polyolefin composition containing a basic polyamide dye site additive which creates in the backing dyeability characteristics which cause the backing material when union dyed, after being tufted with a polyamide or polyester face yarn, to assume sub-

stantially the same shade of color as is assumed by the face yarn when the carpet fabric is dyed in a single bath containing the same dye for both the backing and the face yarns. The term union dyed as used throughout the disclosure of this invention is intended to have the usual definition for goods dyed by a union dyeing process, i.e. a process which is a one-bath process as a result of which the same color or shade can be imparted to two or more textile fibers or yarns in the same piece or material.

Particularly, in the invention, the polyolefin composition used in preparing the filament ribbon from which the carpet backing is woven comprises from about 80 to 99.5% by weight of a stereoregular or isotactic polyolefin and 0.5 to 20% by weight of a basic polyamide comprising the reaction product of an aliphatic dicarboxylic acid or derivative thereof and a polyamine containing not more than two primary amino groups and one or more tertiary amino groups, and wherein said basic polyamide is present in an amount sufficient to provide 0.1 to 1.0% by weight of basic nitrogen in the composition and said basic polyamide has a crystallite melting point in the range 50-250° C. Preferably, the polyamide is one derived by reacting azelaic acid, methyl bis-(3-aminopropyl) amine and hexamethylenediamine. Also, preferably, the polyolefin is selected from linear polyethylene, stereoregular poly-(4-methylpentene-1) and isotactic polypropylene.

#### BRIEF DESCRIPTION OF THE DRAWING

A union dyed tufted carpet made according to the invention is illustrated in FIG. 1 in comparison to a non-union dyed piece of tufted carpet which is illustrated in FIG. 2. In FIG. 1, carpet 1 is shown to have both its woven backing 3 and 3a dyed substantially to the same shade as the face yarn 6 which has been tufted into the backing. The area around 3a has been exposed by pulling out tufts of the material to illustrate the sameness of shade of the backing with the shade of color of the face yarn. FIG. 1 thus graphically illustrates a union dyed product of the invention.

In contrast to FIG. 1, FIG. 2 shows that the woven backing 4 and 4a has a different shade of coloring than does the face yarn 5. The area around 4a has been exposed by pulling out tufts. The product of FIG. 1 is further distinguished over the product illustrated in FIG. 2 in that the woven backing 3a has been woven from a polyolefin-polyamide composition according to the invention, whereas the backing 4a has been woven from 100% isotactic polypropylene filament ribbon.

#### DESCRIPTION OF THE PREFERRED EMBODIMENTS

The polyolefin compositions used in practicing the invention are known compositions and are taught, for example, in U.S. Patent 3,433,853. The basic polyamides and their method of use in preparing the polyolefin compositions used in practicing the present invention also are taught in U.S. 3,433,853 and are incorporated by reference into the present invention as materials useful in the practice in the present invention. The basic polyamides, according to the invention, are condensation polymers which are substantially insoluble in water and which have a crystallite melting point (measured using a Fisher-Johns melting point apparatus) of from about 50° C. to about 250° C. If the crystallite melting point of the basic polymer exceeds about 250° C., the polyolefin composition containing it becomes less easily shaped into uniform articles. These polymers, moreover, do not undergo branching and crosslinking during extrusion of the polyolefin compositions and do not degrade during processing.

Preparation of a typical basic polyamide useful for practice of the present invention is described in Example 1, which follows, and preparation of a typical polypropylene composition comprising a basic polyamide is described in Example 2, which also follows.

Example 1.—A basic polyamide containing tertiary amine groups is prepared from the following ingredients in the indicated proportions:

|                                      | Moles  |
|--------------------------------------|--------|
| 5 Azelaic acid                       | 1.50   |
| Hexamethylenediamine (60% aqueous)   | 0.7875 |
| N,N'-bis-(3-aminopropyl)methyl amine | 0.7875 |

The azelaic acid is placed into a 500-ml. resin kettle equipped with a stainless steel stirrer, take-off condenser, nitrogen inlet, thermometer and addition funnel. The amines are added conjugately to the acid melt (115° C.) with stirring in an atmosphere of nitrogen. The amine addition should take from 20 to 30 minutes. When the amines have been added, the temperature is raised to 175° C. for 2 hours. Finally, a vacuum (50 mm. Hg) is applied for 30 minutes. The product is quickly poured into an aluminum pan and allowed to cool in a desiccator over  $\text{CaSO}_4$ ; in a nitrogen atmosphere. The resulting product is white in color and has a melting point range of 163° C.-167° C. and a relative viscosity (2% solution in 90% formic acid at 25° C.) of 1.64.

A basic polyamide containing secondary amine groups is similarly prepared from the following ingredients:

|                                    | Moles  |
|------------------------------------|--------|
| 25 Sebacic acid                    | 1.50   |
| Hexamethylenediamine (60% aqueous) | 0.7875 |
| Diethylene triamine                | 0.7875 |

The product has a viscosity (2% solution in 90% formic acid at 25° C.) of 1.8 to 1.9.

Example 2.—Polyamides, prepared as above described, are mixed with isotactic polypropylene (polyamide, 7.5 parts; polypropylene, 92.5 parts) and each mixture then extruded at temperatures from about 200-210° C. through a 325 mesh screen and die to form strands which are then fed through cooling water and a cutter to form pellets. The pellets are then used as a textile-forming substance to form filaments in a known way through filament forming dies from a bath of the melted polymer composition. The pelleting operation may, if desired, be omitted and filaments formed directly from the molten blend by use of suitable dies.

In practicing the present invention, a polyolefin-polyamide composition such as that described in Example 2 is extruded and stretch oriented by known means into a ribbon form of filament 100 mils wide and of 1080 denier. The filaments are woven into a primary backing material substantially in the manner described in the Rhodes patent. The fabric so formed is manufactured into carpeting by tufting the backing with, for example, 3700 denier nylon 66 (hexamethylene adipamide) as sold by Du Pont under the trademark Antron Type 846 nylon, using, for example, ten stitches per inch and 6.5 rows per inch of the nylon, forming a pile height of  $\frac{1}{8}$  of an inch. The carpet fabric so formed is preferably beck dyed in rope form by the following general procedure.

Preliminary to the dyeing of the carpeting, the carpet fabric is pre-scoured in a bath containing about 0.5% o.w.g. (on weight of goods) of a non-ionic detergent and about 0.5% o.w.g. of sodium carbonate. Any suitable non-ionic detergent may be used, for example, Triton X-100, an isoctyl phenyl polyethoxy ethanol surfactant. The scouring is carried out at a temperature of 150° F. for about 15 to 20 minutes to remove materials used in finishing the yarn, e.g. lubricants, dust, grime, and so forth, which may be present on the tufted carpeting. The pre-scoured carpeting is then thoroughly rinsed with clear water.

An acid dye bath (used only with nylon face fabric) is prepared by mixing the acid dye to be used with water to obtain a smooth, uniform paste, or by dispersing the acid dye in about five times its weight of surfactant, e.g. a 10% alkyl aryl polyether surfactant sold under the trademark Nacconol SL. The amount of dye used will usually range from about 0.5 to 8% o.w.g., with about

1 to 2% o.w.g. preferred. In either case, the dye mixture obtained is further diluted with bath water equal to from 20 to 100 times the weight of a fabric to be dyed. The ratio of bath liquor to the carpet material in the bath preferably should be about 40 to 1 by weight ratio. Nylon-faced carpet then is placed in a beck apparatus in rope form in about 20 to 100 parts o.w.g. of water. Before mixing the dye concentrate in the water used for the main body of the bath, the bath water is heated to an initial bath temperature of about 100° F. The pH of the bath is adjusted and maintained between 6.5 and 7.5 with a buffer such as monosodium phosphate,  $\text{NaH}_2\text{PO}_4$ . The acid dyestuff, preferably one of the dyes selected from those listed by Color Index Number in Table 2, is dissolved in the bath to make a concentration of dyestuff of 2.0% o.w.g. The temperature of the bath is then raised to about 160 to 170° F. Acidity of the bath is adjusted to a pH of 3.0 to 3.5 with formic acid or an acid forming salt or other organic acid while bringing the bath to a boil at the rates of about 2 to 3 degrees per minute. The dyeing process is carried on for about 1½ hours at a temperature of about 205 to 210° F. The bath is then drawn off and the dyed carpeting is then preferably post-scoured with a scouring bath containing from 0.01 to 5% of a detergent, preferably 0.5% Triton X-100, adjusted with sodium carbonate to a pH 9.5 to 10. The scouring is carried out at 150° F. for about 20 minutes. A union dyed nylon-faced carpet is thus provided.

In practicing the present invention, it has been found that, whereas nylon face yarn may be dyed either by means of an acid dye or a disperse dye, a polyester face yarn must be dyed with a disperse dye in order to get a union shade of color in both the face yarn and the polypropylene-polyamide composition backing. When a disperse dyestuff is to be used, the dyeing procedure is somewhat different from that used in using an acid dyestuff. In either case, the scouring treatments are the same. A bath for dyeing with a disperse dye is prepared substantially as described for the acid bath. Sufficient bath water is provided to establish a ratio of about 40 parts by weight of liquid to one part by weight of carpeting. Polyester-faced carpet is placed in the bath water, preferably in a beck dyeing machine and in rope form. Then 1% o.w.g. of monosodium phosphate is added as a buffer. The bath temperature is raised to about 160° F. To the bath then is added 5% o.w.g. of a carrier, Carolid 3 F (Tanatex Corp.). The bath is then adjusted with acetic acid (1% o.w.g.) to a pH of 5.5 to 6.0. The disperse dyestuff which is to be used to dye the carpet fabric is then introduced into the bath as a concentrate in hot water. The pH is then re-checked and, if necessary, adjusted to the 5.5 to 6.0 range. The temperature of the bath is then raised to the boiling point at a rate of about 3° per minute. The goods are then dyed at the boil for about 60 minutes, or until a uniform depth, i.e. union shade, of color is obtained both in the face yarn and the backing. The dye bath solution is then drained off and the union dyed carpeting is rinsed in hot water at about 160° F., or higher, to remove the residual dye and carrier. The dyed tufted carpeting is given a final rinse in cool water and then dried.

In carrying out the acid dye bath process, it has been found advantageous to start the acid dye cycle at a relatively higher pH in the range of 5.5 to 7.0, and then to lower the pH either incrementally during the dye cycle or, preferably, all at one time after the boiling point has been reached, to a pH of 3.5 or less. This procedure promotes a deeper shade in both the backing and the face yarn and helps to provide a union shade without as much likelihood of obtaining a streaked face yarn as is likely when the dyeing is carried out at a low pH for the entire dye cycle. Disperse dyestuffs which have been found advantageous for producing solid union dyed shades of color in tufted carpeting made and dyed according to the invention are listed in Table 1. It is to

be understood that this list does not include all disperse dyes which may be useful for the practice of the invention, but it is representative of dyes which has been found to provide a union shade in both the face yarn and the backing when the invention is practiced. Acid dyestuffs which may be used in practicing the invention are listed in Table 2.

The amount of disperse dyestuff which will be required in a particular dyeing situation may range from about 0.25 to 3.0% o.w.g. A bath containing 0.5% o.w.g. is especially preferred.

The nylon face yarn of the carpeting preferably is made of nylon 66, a polyamide fiber-forming substance whose chemical composition is hexamethylene adipamide. For acid dyeing, nylon Type 846, sold under the trademark Du Pont, is especially preferred for acid dyeing processes. However, any long chain synthetic polyamide having recurring amide groups



as an integral part of the polymer chain may advantageously be used as the face yarn in the union dyed carpeting of the present invention. Suitable nylon fibers in yarn form for use in the practice of the invention may be selected from those described in "Guidebook to Man-Made Textile Fibers and Textured Yarns of the World," Adeline A. Dembeck, The United Piece Dye Works, New York, N.Y., 3rd edition, pages 136-158, incorporated herein by reference.

The polyester face yarn of the carpeting may be made of a fiber of any long chain synthetic polymer composed of at least 85% by weight of an ester of a dihydric alcohol and terephthalic acid



Suitable polyesters for use in practice of the invention also may be selected from the "Guidebook," supra, pages 172-186 of which are also incorporated herein by reference.

A preferred polyester fiber-forming substance is polyethylene terephthalate fiber, although others may be employed, more specifically those in which the recurring unit in the polyester chain is the diacyl aromatic radical from terephthalic acid, isophthalic acid, 5-t-butylisophthalate, or naphthalene dicarboxylic acids, such as naphthalene-2,6- and naphthalene-2,7-dicarboxylic acids.

The product and process of the present invention are surprising in view of the teachings of U.S. Patent 3,493,316. The patent teaches that when an upholstery fabric was prepared by weaving together five or six different fabric materials, and the composite fabric then is dyed in a dye bath containing a mixture of dispersed and acid dyes, each of the fabric materials assumes a different color. Specifically, the nylon 6 fabric, for example, dyed to a bright red, whereas a mixture of a 30% polyester-70% polyamide blend dyed to a bright orange, a polyethylene terephthalate polyester dyed to a light tan, and a polyacrylonitrile, Orlon 42, dyed to a white, cellulose acetate dyed to a light orange, and silk dyed to a brown. Also, the patent teaches that a four component fabric prepared from nylon 66, nylon 6, 30% polyester-70% polyamide, and 40% polyester-60% polyamide was dyed with disperse dye Blue 3 in a single dye bath at 206° F.; the dyed fabric exhibited four different shades of the same color. Therefore, at the time the present invention was made, it was unexpected that a carpet backing made of polypropylene-polyamide composition containing 0.5 to 20% of a basic polyamide in blended form and tufted with a polyamide face yarn could be dyed in a union bath to a union dye shade in a single dye bath in a single dyeing operation. It was still less expected that the polypropylene-polyamide composition backing when tufted with a polyester face yarn could be dyed to a union dyed

shade in a single dyeing with the same dye in the same dye bath.

The invention is further illustrated in the following examples:

Example 3.—An acid dyeable polyolefin-polyamide composition prepared as described in Examples 1 and 2 above, and as further described in U.S. Patent 3,433,853, supra, was extruded into 500 denier XR ribbon and 1100 denier XR ribbon. The ribbon was woven into a closed weave fabric and tufted with Du Pont Antron Type 846 regular dyeing carpet nylon 66 (hexamethylene adipamide). The tufted carpet was scoured as discussed above and acid dyed in a mixture of acid dyes in accordance with the general procedure also discussed above. The acid dyestuffs used consisted of 1.65% Mercacyl Yellow 4 G, 0.05% Mercacyl Blue 2 GA, and 0.18% Nylomene Red B3BS, all percentages being based on the weight of the carpet material. The bath was prepared in a beck apparatus using 1% o.w.g. Alkanol ND (Du Pont) as a surfactant and 2% o.w.g. of monosodium phosphate as a buffer. The bath contained about 40 parts water per one part of carpet by weight. The carpeting was placed in the beck in rope form. The temperature of the bath was raised to the boiling point at about 3° per minute. The pH of the bath at this point was determined to be about 5.5 to 6.0. After 15 minutes at a boil, the bath was adjusted to a pH of 4.0 with formic acid. After another 15 minutes of boiling, the bath was adjusted to 3.5. The carpeting material then was dyed at the boil for 15 minutes of additional time. The bath water was then dropped and the dyed carpet was rinsed with water at 160° F. until clear. The carpet was then dried. The dyed tufted carpet was found to have the face yarn dyed to a uniform gold shade with the backing dyed to a satisfactory union gold shade.

Example 4.—A woven fabric was prepared as in Example 3 and was then tufted with a regular dyeing spun polyester carpet yarn. A bath for beck dyeing of the tufted carpet with a disperse dyestuff was prepared using 40 parts water per one part of carpet by weight. The carpet was placed in the beck in rope form. The bath temperature was set at 100° F. Synthropol PWS (1% o.w.g.) (ethylene oxide condensate, nonionic surfactant) was added. A mixture of disperse dyestuffs was prepared in water solution. The mixture consisted of 0.14% Calcosyn Blue RP, 0.26% Latyl Orange 3 R, and 0.80% Setacyl Yellow P-GSL. The dyestuff mixture was added to the bath and the bath stirred until the dyestuff had been thoroughly dispersed. The temperature of the bath was then raised to 170° F. Then, 10% o.w.g. of Carolid 3 F carrier (chlorinated phenolic) (Tatanex Corporation) was added. The temperature was raised to the boiling point of the bath, and the carpeting was dyed at the boil for 45 minutes. The bath was then dropped and the dyed carpeting was rinsed and dried in the usual manner. The face yarn of the tufted carpet was found to be dyed to a uniform gold shade and the backing was dyed to a satisfactory union dye gold shade.

Examples 5-30.—Fabrics prepared as in Example 3 and tufted with a regular dyeing polyester fiber face yarn were used to make test pieces of tufted fabric which were laboratory dyed by the disperse dye dyeing procedure of Example 4. The disperse dyestuffs which were used and the amounts thereof, as well as the color rating which were determined, are shown in Table 1, Examples 5-30.

Examples 31-35.—Fabrics were prepared as described in Example 3 and tufted with Du Pont Antron Type 846 nylon 66 face yarn. The carpet fabrics so prepared were dyed with a disperse dye. Each fabric was first pre-scoured with a water solution containing 0.5% o.w.g. of a non-ionic detergent, Triton X-100, and 1% o.w.g. of sodium carbonate, at 152 to 160° F. for 20 minutes to remove finish, lubricant, dust, and other contaminants. A dye bath was then prepared in a beck apparatus using 40 parts liquid to one part by weight of the carpet fabric. The

fabric was placed in the beck in rope form. The bath was heated to 100° F. and 1% o.w.g. of a detergent, Merpol DA (ethylene oxide condensate, Du Pont) and 1% o.w.g. of trisodiumpyrophosphate were added. A disperse dyestuff selected from those shown in Table 1, Examples 31-35, was used to make a dye concentrate. The dye concentrate was added to the dyestuff in the amount of 0.5% o.w.g. The bath temperature was raised to about 205 to 200° F. at the rate of about 3° per minute. The dyeing operation was carried on for about 60 minutes. The bath was then drained off and the dyed carpet fabric was rinsed and the carpeting dried. The results obtained are shown in Table 1 under the heading Color Rating. Each dyed sample was at or near a union dye shade. The term "near union shade" is intended to mean that the shade of the backing and face yarn in each case were close enough to make the fabric acceptable for carpeting for home and office use.

Examples 36-46.—Fabric prepared as described in Example 3 and tufted with Du Pont Antron Type 846 regular dyeing carpet nylon 66 was acid dyed using acid dyestuffs. The fabric was pre-scoured with a water solution containing 0.5% non-ionic detergent and 0.5% of sodium carbonate in the form of soda ash. Triton X-100 was used as the detergent. A dye bath was prepared using 40 parts liquid per one part by weight of fabric. The tufted fabric was placed in a beck in rope form. The bath was set at 100° F. and 1% o.w.g. of Alkanol ND and 2% o.w.g. of monosodium phosphate were added. An acid dyestuff selected from the dyestuffs shown in Table 2 was added to the bath in about 2% o.w.g. The temperature of the bath was raised to a boil at the rate of 2 to 3° per minute. As the fabric was being dyed, the pH was adjusted to the range of 3.0 to 3.5 with formic acid. Dyeing was carried out at a temperature of about 205 to 210° F. over a 1½ hour period. The bath was then dropped and the dyed fabric was rinsed. The results obtained are shown in Table 2 under the heading Color Rating. It is shown that a union shade or near union shade was obtained in each dyeing.

Example 47.—A tufted carpet prepared as described in Examples 36-46 was dyed in the manner described in Examples 36-46 using a mixture of dyestuffs comprising or consisting of 0.14% of Calcosyn Blue RP (Disperse Blue 116), 0.26% Latyl Orange 3 R (Disperse Orange 21), and 0.80% Setacyl Yellow P-GSL (Disperse Yellow 50). The dyed tufted carpet was found to have the nylon 66 face yarn dyed a uniform gold shade and the backing dyed to a union shade of gold.

While the invention has been described in relation to a union dyed tufted carpet fabric, it will be obvious to those skilled in the art that the invention can be practiced to union dye fabrics prepared for other use or constructed in other ways than by tufting a face yarn into a woven backing. For example, a woven fabric may be made by interweaving a polyester yarn or a polyamide yarn with a yarn or with ribbons or filaments of the polyolefin-polyamide composition used to practice the present invention, and then dyed to a union shade with an acid or disperse dye according to the procedures of the examples disclosed above.

Also, although the polyolefin-polyamide composition has been described in its filamentary ribbon textile-forming form, the composition also can be used to make a union dyed fabric having a non-woven fabric or film form of the union dyed, polyolefin-polyamide composition backing tufted with a polyamide or polyester fiber yarn and union dyed according to the invention.

The term fiber as used in describing the invention includes and is intended to include filaments of round, rectangular, oval, or other known cross-sectional forms, whether the fiber is in continuous or discontinuous, e.g. chopped, fibrous form. The term yarn likewise includes and is intended to include textured and non-textured yarns made of the above-described fibers.

TABLE 1.—DISPERSE DYESTUFFS

| Ex. No. | Dyestuff name           | Color index number <sup>1</sup>     | Face yarn                          | Dyestuff used, percent o.w.g. | Color rating            |
|---------|-------------------------|-------------------------------------|------------------------------------|-------------------------------|-------------------------|
| 5       | Latyl Yellow RC         | Disperse Yellow 8, C.I. No. 12690.  | ENCRON Polyester                   | .5                            | At or near union shade. |
| 6       | Latyl Yellow 4RL        | Disperse Yellow 23, C.I. No. 26070. | do                                 | .5                            | Do.                     |
| 7       | Latyl Yellow YLW        | Disperse Yellow 42, C.I. No. 10338. | Blue "C" Polyester                 | .5                            | Do.                     |
| 8       | Latyl Yellow 3G         | Disperse Yellow 54                  | ENCRON Polyester                   | .5                            | Do.                     |
| 9       | Latyl Orange NST        | Disperse Orange 25                  | Blue "C" Polyester                 | .5                            | Do.                     |
| 10      | Latyl Orange 3R         | Disperse Orange 26                  | do                                 | .5                            | Do.                     |
| 11      | Latyl Yellow RSF        | Disperse Orange 40                  | ENCRON Polyester                   | .5                            | Do.                     |
| 12      | Latyl Yellow 5R         | Disperse Orange 41                  | do                                 | .5                            | Do.                     |
| 13      | Latyl Cerise Y          | Disperse Red 55                     | do                                 | .5                            | Do.                     |
| 14      | Latyl Scarlet FSW       | Disperse Red 56                     | do                                 | .5                            | Do.                     |
| 15      | Latyl Cerise B          | Disperse Red 59                     | Blue "C" Polyexter                 | .5                            | Do.                     |
| 16      | Latyl Cerise N          | Disperse Red 60                     | do                                 | .5                            | Do.                     |
| 17      | Latyl Red MG            | Disperse Red 65                     | ENCRON Polyester                   | .5                            | Do.                     |
| 18      | Latyl Red GFS           | Disperse Red 88                     | do                                 | .5                            | Do.                     |
| 19      | Latyl Red B             | Disperse Violet 17                  | do                                 | .5                            | Do.                     |
| 20      | Latyl Violet 2R         | Disperse Violet 18                  | Blue "C" Polyester                 | .5                            | Do.                     |
| 21      | Latyl Bordeaux B        | Disperse Violet 26                  | do                                 | .5                            | Do.                     |
| 22      | Latyl Violet BN         | Disperse Violet 27                  | do                                 | .5                            | Do.                     |
| 23      | Latyl Blue FLW          | Disperse Blue 27, C.I. No. 60767.   | do                                 | .5                            | Do.                     |
| 24      | Latyl Blue BCN          | Disperse Blue 59                    | do                                 | .5                            | Do.                     |
| 25      | Latyl Brilliant Blue BG | Disperse Blue 60                    | ENCRON Polyester                   | .5                            | Do.                     |
| 26      | Latyl Blue LS           | Disperse Blue 62                    | Blue "C" Polyester                 | .5                            | Do.                     |
| 27      | Latyl Blue 2R           | Disperse Blue 63                    | ENCRON Polyester                   | .5                            | Do.                     |
| 28      | Latyl Blue 4R           | Disperse Blue 64                    | Blue "C" Polyester                 | .5                            | Do.                     |
| 29      | Latyl Blue RB           | Disperse Blue 65                    | ENCRON Polyester                   | .5                            | Do.                     |
| 30      | Latyl Brown MS          | Disperse Brown 2                    | do                                 | .5                            | Do.                     |
| 31      | Latyl Violet BN         | Disperse Violet 27                  | DU PONT'S ANTRON Type 846 nylon 66 | .5                            | Do.                     |
| 32      | Latyl Bordeaux B        | Disperse Violet 26                  | do                                 | .5                            | Do.                     |
| 33      | Latyl Yellow 4RL        | Disperse Yellow 23                  | do                                 | .5                            | Do.                     |
| 34      | Latyl Red MG            | Disperse Red 65                     | do                                 | .5                            | Do.                     |
| 35      | Latyl Yellow 3G         | Disperse Yellow 54                  | do                                 | .5                            | Do.                     |

<sup>1</sup> The Colour Index, Textile Chemist and Colorist, Products-70, September 1969, vol. No. 20A, Jour. AATCC.

TABLE 2.—ACID DYESTUFFS

| Ex. No. | Dyestuff name      | Color index number            | Dyestuff used, percent o.w.g. | Color rating      |
|---------|--------------------|-------------------------------|-------------------------------|-------------------|
| 36      | Merpacyl Blue SW   | Acid Blue 25, C.I. No. 62055. | 2.0                           | At union shade.   |
| 37      | Merpacyl Blue SK   | Acid Blue 78, C.I. No. 62105. | 2.0                           | Do.               |
| 38      | Merpacyl Blue 2GA  | Acid Blue 40, C.I. No. 62125. | 2.0                           | Near union shade. |
| 39      | Merpacyl Yellow AR | Acid Orange 132               | 2.0                           | At union shade.   |
| 40      | Merpacyl Yellow G  | Acid Yellow 175               | 2.0                           | Do.               |
| 41      | Merpacyl Yellow 4G | Acid Yellow 174               | 2.0                           | Do.               |
| 42      | Merpacyl Yellow 8G | Acid Yellow                   | 2.0                           | Do.               |
| 43      | Merpacyl Orange R  | Acid Orange 128               | 2.0                           | Do.               |
| 44      | Merpacyl Red G     | Acid Red 337                  | 2.0                           | Do.               |
| 45      | Merpacyl Red L     | Acid Red 151, C.I. No. 26900. | 2.0                           | Do.               |
| 46      | Merpacyl Red B     | Acid Red 236                  | 2.0                           | Do.               |

<sup>1</sup> Du Pont's ANTRON Type 846.

I claim:

1. A process for preparing a union dyed fabric, said process comprising  
union dyeing in a dye bath selected from acid dye baths  
and disperse dye baths a synthetic fabric containing  
synthetic fibers selected from the group consisting of  
polyamide and polyester fibers in a fiber blend with  
fibers of a polyolefin composition,  
said polyamide consisting of a long chain synthetic  
polyamide having recurring amide groups



as an integral part of the polymer chain,  
said polyester being a long chain synthetic polymer  
composed of at least 85% by weight of an ester of a  
dihydric alcohol and terephthalic acid



and  
said composition comprising 80-99.5% by weight of a  
stereoregular polyolefin and 0.5 to 20% by weight of

55  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635<br

## 11

acid dye bath and the synthetic fiber-forming substance is a polyamide.

7. The process of claim 1 wherein the dye bath is a disperse dye bath.

8. A union dyed tufted textile fabric comprising

5

(a) a backing consisting of fibers of a polyolefin composition, said composition comprising 80-99.5% by weight of a stereoregular polyolefin and 0.5 to 20% by weight of a basic polyamide comprising the reaction product of an aliphatic dicarboxylic acid for derivative thereof and a polyamine containing not more than two primary amino groups and one or more tertiary amino groups, wherein said basic polyamide is present in an amount sufficient to provide 0.1 to 1.0% by weight of basic nitrogen in the composition and said basic polyamide has a crystallite melting point in the range 50-250° C.,

15

(b) face yarn consisting of synthetic fibers selected from the group consisting of polyamide and polyester fibers, said polyamide consisting of a long chain synthetic polyamide having recurring amide groups



as an integral part of the polymer chain, said polyester being a long chain synthetic polymer composed of at least 85% by weight of an ester of a dihydric alcohol and terephthalic acid

25



30

and

(c) a union shade of color in both said backing and face yarn provided from at least one synthetic dye selected from acid dyes and disperse dyes, wherein said acid dyes are used only with the polyamide face yarn, and the disperse dyes are used with both the polyamide and polyester face yarns.

9. The union dyed tufted fabric of claim 8 wherein the polyamide is hexamethylene adipamide.

10. The union dyed tufted fabric of claim 8 wherein the polyester is polyethylene terephthalate.

11. The union dyed tufted fabric of claim 8 wherein the polyolefin is selected from the group consisting of linear polyethylene, stereoregular poly-(4-methylpentene-1) and isotactic polypropylene.

12. The union dyed tufted fabric of claim 8 wherein the polyamine consists of a mixture of methyl bis(3-aminopropyl) amine and hexamethylenediamine.

13. The union dyed tufted fabric of claim 8 wherein the polyolefin is isotactic polypropylene.

14. A union dyed textile fabric comprising

(a) fibers of a polyolefin composition, said composition

## 12

comprising 80-99.5% by weight of a stereoregular polyolefin and 0.5 to 20% by weight of a basic polyamide comprising the reaction product of an aliphatic dicarboxylic acid for derivative thereof and a polyamine containing not more than two primary amino groups and one or more tertiary amino groups, wherein said basic polyamide is present in an amount sufficient to provide 0.1 to 1.0% by weight of basic nitrogen in the composition and said basic polyamide has a crystallite melting point in the range 50-250° C.,

(b) synthetic fibers selected from the group consisting of polyamide and polyester fibers, said polyamide consisting of a long chain synthetic polyamide having recurring amide groups



as an integral part of the polymer chain, said polyester being a long chain synthetic polymer composed of at least 85% by weight of an ester of a dihydric alcohol and terephthalic acid



and

(c) a union shade of color in both said composition and fibers provided from at least one synthetic dye selected from acid dyes and disperse dyes, wherein said acid dyes are used only with the polyamide fibers, and the disperse dyes are used with both the polyamide and polyester fibers.

## References Cited

## UNITED STATES PATENTS

|           |         |              |       |         |
|-----------|---------|--------------|-------|---------|
| 3,485,569 | 12/1969 | Newby et al. | ----- | 8-21 B  |
| 3,433,853 | 3/1969  | Earle et al. | ----- | 260-857 |
| 3,361,843 | 1/1968  | Miller       | ----- | 260-857 |
| 3,439,999 | 4/1969  | Miller       | ----- | 8-15    |
| 3,485,574 | 12/1969 | Miller       | ----- | 8-168 X |

## OTHER REFERENCES

Cuthbertson et al.: The Textile Manufacturer, September 1964, pp. 353-359.

DONALD LEVY, Primary Examiner

U.S. CL. X.R.

8-21 C; 57-140 B; 161-62

50